



US011920307B2

(12) **United States Patent**  
**Sachs et al.**

(10) **Patent No.:** US 11,920,307 B2  
(45) **Date of Patent:** \*Mar. 5, 2024

(54) **MULTI-PLY TISSUE PRODUCTS HAVING IMPROVED CROSS-MACHINE DIRECTION PROPERTIES**

(71) Applicant: **Kimberly-Clark Worldwide, Inc.**, Neenah, WI (US)

(72) Inventors: **Mark W. Sachs**, Appleton, WI (US); **Richard A. Zanon**, Appleton, WI (US); **Lynda E. Collins**, Neenah, WI (US); **Kevin J. Vogt**, Neenah, WI (US); **Christopher L. Satori**, Hortonville, WI (US)

(\*) Notice: Subject to any disclaimer, the term of this patent is extended or adjusted under 35 U.S.C. 154(b) by 0 days.

This patent is subject to a terminal disclaimer.

(21) Appl. No.: **17/869,481**

(22) Filed: **Jul. 20, 2022**

(65) **Prior Publication Data**

US 2022/0364311 A1 Nov. 17, 2022

**Related U.S. Application Data**

(63) Continuation of application No. 17/007,394, filed on Aug. 31, 2020, now Pat. No. 11,427,967.

(51) **Int. Cl.**

**D21H 27/00** (2006.01)  
**D21F 11/00** (2006.01)  
**D21H 27/40** (2006.01)

(52) **U.S. Cl.**

CPC ..... **D21H 27/005** (2013.01); **D21F 11/006** (2013.01); **D21H 27/40** (2013.01)

(58) **Field of Classification Search**

CPC ..... D21H 27/005; D21H 27/40; D21F 11/006  
See application file for complete search history.

(56) **References Cited**

U.S. PATENT DOCUMENTS

4,440,597 A 4/1984 Wells et al.  
4,638,907 A 1/1987 Bedenk et al.  
(Continued)

FOREIGN PATENT DOCUMENTS

EP 0625610 A1 11/1994  
EP 2334868 B1 4/2017  
(Continued)

OTHER PUBLICATIONS

Tissue360.tappi, "Sheet Structure Process Effect on Tissue Properties", <https://tissue360.tappi.org/>.

*Primary Examiner* — Eric Hug

*Assistant Examiner* — Matthew M Eslami

(74) *Attorney, Agent, or Firm* — KIMBERLY-CLARK WORLDWIDE, INC.

(57) **ABSTRACT**

Provided are tissue webs, and products produced therefrom, that are generally durable, flexible and have improved cross-machine direction (CD) properties, such as CD tensile energy absorption (CD TEA), CD stretch and CD modulus. The inventive tissue products generally comprise multiple tissue plies, such as two or more plies, that have been prepared by through-air drying and more preferably by through-air drying without creping. Moreover, the plies may be produced in a through-air drying process that utilizes a transfer fabric positioned between the forming fabric and the through-air drying fabric where the transfer fabric imparts the nascent web with a high degree of CD strain.

13 Claims, 5 Drawing Sheets



| (56)                     | References Cited |                                                            |
|--------------------------|------------------|------------------------------------------------------------|
| U.S. PATENT DOCUMENTS    |                  |                                                            |
| 5,591,309 A              | 1/1997           | Rugowski et al.                                            |
| 5,607,551 A              | 3/1997           | Farrington, Jr. et al.                                     |
| 5,656,132 A              | 8/1997           | Farrington, Jr. et al.                                     |
| 5,672,248 A              | 9/1997           | Wendt et al.                                               |
| 5,746,887 A              | 5/1998           | Wendt et al.                                               |
| 5,772,845 A              | 6/1998           | Farrington, Jr. et al.                                     |
| 5,830,321 A              | 11/1998          | Lindsay et al.                                             |
| 6,017,417 A              | 1/2000           | Wendt et al.                                               |
| 6,585,856 B2             | 7/2003           | Zwick et al.                                               |
| 6,827,818 B2             | 12/2004          | Farrington, Jr. et al.                                     |
| 6,887,348 B2             | 5/2005           | Hermans et al.                                             |
| 6,893,535 B2             | 5/2005           | Hermans et al.                                             |
| 7,166,189 B2             | 1/2007           | Burazin et al.                                             |
| 7,294,229 B2             | 11/2007          | Hada et al.                                                |
| 7,399,378 B2             | 7/2008           | Edwards et al.                                             |
| 7,497,925 B2             | 3/2009           | Hermans et al.                                             |
| 7,611,605 B2             | 11/2009          | Burazin et al.                                             |
| 7,726,349 B2             | 6/2010           | Mullally et al.                                            |
| 7,828,932 B2             | 11/2010          | Hermans et al.                                             |
| 7,935,220 B2             | 5/2011           | Edwards et al.                                             |
| 7,935,221 B2             | 5/2011           | Allen et al.                                               |
| 7,935,409 B2             | 5/2011           | Burazin et al.                                             |
| 7,938,932 B2             | 5/2011           | Hermans et al.                                             |
| 7,972,474 B2             | 7/2011           | Underhill et al.                                           |
| 8,481,133 B2             | 7/2013           | Hermans et al.                                             |
| 8,574,399 B2             | 11/2013          | Hermans et al.                                             |
| 8,652,597 B2             | 2/2014           | Hermans et al.                                             |
| 8,852,398 B2             | 10/2014          | Hermans et al.                                             |
| 8,940,376 B2             | 1/2015           | Stage et al.                                               |
| 8,956,503 B2             | 2/2015           | Hermans et al.                                             |
| 9,222,224 B2             | 12/2015          | Shannon                                                    |
| 10,161,084 B2            | 12/2018          | Burazin et al.                                             |
| 11,286,623 B2            | 3/2022           | Sachs et al.                                               |
| 11,299,856 B2            | 4/2022           | Sachs et al.                                               |
| 2003/0136529 A1          | 7/2003           | Burazin et al.                                             |
| 2004/0118544 A1          | 6/2004           | Tirimacco et al.                                           |
| 2004/0200590 A1          | 10/2004          | Wilhelm                                                    |
| 2005/0133175 A1          | 6/2005           | Hada et al.                                                |
| 2005/0145352 A1          | 7/2005           | Hermans et al.                                             |
| 2005/0145353 A1          | 7/2005           | Troxell et al.                                             |
| 2005/0148257 A1          | 7/2005           | Hermans et al.                                             |
|                          |                  | 2005/0161179 A1 7/2005 Hermans et al.                      |
|                          |                  | 2005/0236122 A1 10/2005 Mullally et al.                    |
|                          |                  | 2005/0241786 A1 11/2005 Edwards et al.                     |
|                          |                  | 2006/0086472 A1 4/2006 Hermans et al.                      |
|                          |                  | 2006/0130986 A1 6/2006 Flugge-Berendes et al.              |
|                          |                  | 2007/0000629 A1 1/2007 Tirimacco et al.                    |
|                          |                  | 2007/0131366 A1* 6/2007 Underhill ..... D21F 11/14 162/109 |
|                          |                  | 2007/0137807 A1 6/2007 Schulz et al.                       |
|                          |                  | 2008/0073047 A1 3/2008 Bakken et al.                       |
|                          |                  | 2009/0065160 A1 3/2009 Hermans et al.                      |
|                          |                  | 2009/0194244 A1 8/2009 Harper et al.                       |
|                          |                  | 2010/0051217 A1 3/2010 Allen et al.                        |
|                          |                  | 2011/0155337 A1 6/2011 Murray et al.                       |
|                          |                  | 2012/0247698 A1 10/2012 Murray et al.                      |
|                          |                  | 2013/0160960 A1* 6/2013 Hermans ..... D21H 27/005 162/205  |
|                          |                  | 2014/0118544 A1 5/2014 Asaka et al.                        |
|                          |                  | 2014/0209264 A1 7/2014 Tirimacco et al.                    |
|                          |                  | 2017/0049280 A1 2/2017 Weaver et al.                       |
|                          |                  | 2018/0135248 A1 5/2018 Collins et al.                      |
|                          |                  | 2018/0142421 A1 5/2018 Rouse et al.                        |
|                          |                  | 2018/0195239 A1 7/2018 Ziegenbein                          |
|                          |                  | 2018/0334778 A1 11/2018 Shannon et al.                     |
|                          |                  | 2019/0127919 A1 5/2019 Burazin et al.                      |
|                          |                  | 2019/0264395 A1 8/2019 Rouse et al.                        |
|                          |                  | 2020/0173114 A1 6/2020 Vogt et al.                         |
|                          |                  | 2020/0270812 A1 8/2020 Holz et al.                         |
|                          |                  | 2021/0140119 A1 5/2021 Vogt et al.                         |
|                          |                  | 2021/0207327 A1 7/2021 Margo Moreno et al.                 |
|                          |                  | 2021/0321831 A1 10/2021 Vogt et al.                        |
|                          |                  | 2022/0010496 A1 1/2022 Tirimacco et al.                    |
|                          |                  | 2022/0064863 A1 3/2022 Sachs et al.                        |
|                          |                  | 2022/0064864 A1 3/2022 Sachs et al.                        |
|                          |                  | 2022/0186442 A1 6/2022 Sachs et al.                        |
|                          |                  | 2022/0372703 A1 11/2022 Collins et al.                     |
| FOREIGN PATENT DOCUMENTS |                  |                                                            |
|                          | WO               | 2000008253 A1 2/2000                                       |
|                          | WO               | 2007078562 A2 7/2007                                       |
|                          | WO               | 2010023616 A2 3/2010                                       |
|                          | WO               | 2013041989 A2 3/2013                                       |

\* cited by examiner



FIG. 1



FIG. 2



FIG. 3



FIG. 4



FIG. 5

## 1

**MULTI-PLY TISSUE PRODUCTS HAVING  
IMPROVED CROSS-MACHINE DIRECTION  
PROPERTIES**

**RELATED APPLICATIONS**

The present application is a continuation application and claims priority to U.S. patent application Ser. No. 17/007,394, filed on Aug. 31, 2020, which is incorporated herein by reference.

**BACKGROUND**

Generally, papermakers, particularly manufacturers of low basis weight tissue products, have attempted to improve product softness and durability by altering certain machine and cross-machine direction properties such as tensile strength, stretch and modulus. Of particular interest are cross-machine direction (CD) properties, such as CD tensile energy absorption (CD TEA), CD stretch and CD modulus, because tissue products are typically weakest in the cross-machine direction and most in-use failures occur in this direction. For example, U.S. Pat. No. 7,972,474 to Underhill sought to improve CD properties by manufacturing tissue products using a through-air drying process in which the transfer fabric and the through-air drying fabric were both textured fabrics having a substantially uniform high strain distribution in the cross-machine direction. The resulting tissue products, while having improved cross-machine direction properties such as low modulus and relatively high stretch, were relatively weak in the cross-machine direction, such as CD tensile strengths less than about 600 g/3".

In other instances, tissue makers have altered manufacturing processes to produce products having low degrees of CD modulus. While a low modulus may reduce the perception of the tissue as being stiff, at some point a low CD modulus may be interpreted as indicative of a weak or "flimsy" tissue. This is particularly true when low CD modulus is accompanied by a relatively low CD tensile strength, such as less than about 600 g/3". Thus, in certain instances tissue makers have attempted to increase CD modulus at a given tensile strength. For example, U.S. Pat. No. 7,300,543 to Mullally utilized papermaking fabrics with deep discontinuous pockets in an uncreped through-air dried tissue process to produce tissue products having the desired CD slope values. Similarly, U.S. Pat. No. 8,500,955 to Hermans attempted to improve CD slope at a given CD tensile strength by rewetting the dried tissue web, pressing the rewetted web and then drying the web for a second time.

While tissue makers have been able to modulate certain cross-machine properties they have not succeeded in balancing all of the properties to produce a tissue product that has sufficient strength to withstand use but is also soft and pliable. Therefore, there remains a need in the art for tissue webs and products having balanced cross-machine direction properties and methods of manufacturing the same.

**SUMMARY**

The present inventors have now discovered that various tissue manufacturing techniques, such as wet molding, may be used to create a multi-ply tissue product that is both aesthetically pleasing and has improved physical attributes. For example, the present invention provides a tissue product that has been manufactured by a process, such as through-air drying, which molds the nascent web prior to it being transferred to a through-air drying fabric and dried. The

## 2

inventive tissue products have improved cross-machine direction (CD) properties, such as CD tensile energy absorption (CD TEA), CD stretch and CD modulus, measured as CD Slope. In particularly preferred embodiments the inventive products comprise two or more tissue plies that have been produced by through-air drying without creping, commonly referred to uncreped through-air dried (UCTAD).

In one particularly preferred embodiment the tissue webs of the present invention are manufactured by transferring a 10 partially dewatered web to a transfer fabric, particularly a highly structured transfer fabric, that molds the partially dewatered web prior to it being transferred to a through-air drying fabric. Surprisingly, molding imparted by the transfer fabric is retained in the dried web the resulting tissue 15 products have improved physical properties such as CD TEA, CD stretch and CD modulus, measured as CD Slope.

In other embodiments the present invention provides a multi-ply tissue product having a CD stretch of about 13.0 percent or greater, such as about 13.5 percent or greater, such 20 as about 14.0 percent or greater, such as from about 13.0 to about 15.0 percent. Surprisingly, the foregoing CD Stretch values may be achieved without creping the tissue web. Rather than crepe the web during manufacture, the instant 25 tissue products may be produced by transferring a partially dewatered web to a transfer fabric having a high degree of topography to strain the nascent sheet in the cross-machine direction.

In other embodiments the present invention provides a multi-ply tissue product comprising two through-air dried 30 tissue plies, the product having a CD tensile strength of about 2,500 g/3" or greater, such as about 2,750 g/3" or greater, such as about 3,000 g/3" or greater, such as from about 2,500 to about 3,750, such as from about 2,750 to about 3,500 g/3", such as from about 3,000 to about 3,300 g/3" and a CD stretch from about 13.0 to about 15.0 percent.

In still other embodiments the present invention provides a multi-ply tissue product having a CD Tensile from about 3,000 to about 3,500 g/3" and a CD TEA of about 25.0 g·cm/cm<sup>2</sup> or greater, such as about 28.0 g·cm/cm<sup>2</sup> or greater, such as about 30.0 g·cm/cm<sup>2</sup> or greater, such as from about 40 25.0 to about 34.0 g·cm/cm<sup>2</sup>. In certain embodiments the inventive tissue products may have a CD TEA Index of about 10.0 or greater, such as about 10.5 or greater, such as about 11.0 or greater, such as from about 10.0 to about 12.0.

In another embodiment, tissue products of the present invention have sufficient strength to maintain integrity in-use but are flexible and soft. For example, the products may have a geometric mean tensile strength (GMT) from about 45 2,500 to about 3,500 g/3" and a CD Slope less than about 15.0 kg, such as from about 7.5 to about 15.0 kg, such as from about 7.5 to about 12.0 kg.

In still other embodiments the inventive tissue products are able to absorb a large amount of energy in the cross-machine direction before rupturing. For example, the inventive 55 tissue products may have a high degree of CD Stretch, such as about 13.0 percent or greater, such as about 13.5 percent or greater, such as about 14.0 percent or greater, such as from about 13.0 to about 15.0 percent and a CD Slope less than about 15.0 kg.

In still other embodiments the present invention provides a method of manufacturing a multi-ply tissue product comprising two through-air dried tissue plies having improved cross-machine direction properties comprising the steps of dispersing papermaking fibers in water to form an aqueous 60 suspension of fibers; depositing the aqueous suspension of fibers on a forming fabric to form a wet tissue web; partially dewatering the wet tissue web; transferring the partially

dewatered tissue web to a transfer fabric having CD strain from about 15 to about 19 percent; transferring the molded tissue web to a through-air drying fabric; conveying the tissue web over a dryer while supported by the through-air drying fabric to dry the tissue web to a consistency of at least about 95 percent; and plying two dried tissue webs together in facing arrangement.

#### BRIEF DESCRIPTION OF DRAWINGS

FIG. 1 is a graph of geometric mean tensile (x-axis) versus CD Stretch (y-axis) for inventive (●) and commercial (▲) tissue products;

FIG. 2 is a graph of CD tensile (x-axis) versus CD Slope (y-axis) for inventive (●) and commercial (▲) tissue products;

FIG. 3 is a graph of CD tensile (x-axis) versus CD Slope (y-axis) for inventive (●) and commercial (▲) tissue products;

FIG. 4 illustrates one embodiment for forming a basesheet useful in the production of a tissue product according to the present invention; and

FIG. 5 is profilometry scan of a transfer fabric useful in the manufacture of tissue products according to the present invention.

#### DEFINITIONS

As used herein the term “Basesheet” refers to a tissue web formed by any one of the papermaking processes described herein that has not been subjected to further processing, such as embossing, calendering, treatment with a binder or softening composition, perforating, plying, folding, or rolling into individual rolled products.

As used herein the term “Tissue Product” refers to products made from basesheets and includes, bath tissues, facial tissues, paper towels, industrial wipers, foodservice wipers, napkins, medical pads, and other similar products.

As used herein the term “Ply” refers to a discrete tissue web used to form a tissue product. Individual plies may be arranged in juxtaposition to each other. In a preferred embodiment, tissue products prepared according to the present invention comprise multiple plies, such as two or more plies.

As used herein, the term “Layer” refers to a plurality of strata of fibers, chemical treatments, or the like, within a ply. A “Layered Tissue Web” generally refers to a tissue web formed from two or more layers of aqueous papermaking furnish. In certain instances, the aqueous papermaking furnish forming two or more of the layers comprises different fiber types.

As used herein the term “Machine Direction” (MD) generally refers to the direction in which a tissue web or product is produced. The term “Cross-Machine Direction” (CD) refers to the direction perpendicular to the machine direction.

As used herein, the term “Papermaking Fabric” means any fabric useful in the manufacture of a fibrous structure, such as a tissue sheet, typically by a wet-laid process. Specific papermaking fabrics within the scope of this invention include transfer fabrics for conveying a wet web from one papermaking step to another, such as described in U.S. Pat. No. 5,672,248 and through-air drying fabric for supporting a web as it is transported over one or more through-air dyers, such as described in U.S. Pat. Nos. 5,429,686, 6,808,599 and 6,039,838.

As used herein the term “Machine Direction Oriented” when referring to a protuberance on a papermaking fabric generally means that the element or protuberance’s principle axis of orientation is positioned at an angle of less than about 20 degrees relative to the machine direction (MD) axis of the fabric or tissue sheet.

As used herein the term “Cross-Machine Direction Oriented” when referring to a protuberance on a papermaking fabric generally means that the element or protuberance’s principle axis of orientation is positioned at an angle of greater than about 20 degrees relative to the machine direction (MD) axis of the fabric or tissue sheet. For example, a discrete, nonwoven protuberance disposed on the web contacting surface of a papermaking fabric having an element angle greater than 20 degrees, such as from 20 to about 40 degrees, may be said to be cross-machine direction oriented.

As used herein, the term “Protuberance” generally refers to a three-dimensional element disposed on the web contacting surface of a papermaking fabric. For example, in one embodiment, a protuberance may be formed by one or more warp filaments overlaying a plurality of shute filaments. In other instances, a protuberance may be a nonwoven material disposed on the web contacting surface of the fabric.

As used herein, the term “Valley” generally refers to a portion of a papermaking fabric that lies below the uppermost surface plane of the fabric and is generally bounded by a pair of spaced apart protuberances.

As used herein the term “Basis Weight” generally refers to the conditioned weight per unit area of a tissue and is generally expressed as grams per square meter (gsm). Basis weight is measured as described in the Test Methods section below. While the basis weights of tissue products prepared according to the present invention may vary, in certain embodiments the products have a basis weight of about 45.0 gsm or greater, such as about 48.0 gsm or greater, such as 50.0 gsm or greater, such as from about 45.0 to about 55.0 gsm, such as from about 48.0 to about 52.0 gsm.

As used herein, the term “Caliper” refers to the thickness of a tissue product, web, sheet or ply, typically having units of microns ( $\mu\text{m}$ ) and is measured as described in the Test Methods section below.

As used herein, the term “Sheet Bulk” refers to the quotient of the caliper ( $\mu\text{m}$ ) divided by the basis weight (gsm) and having units of cubic centimeters per gram (cc/g). Tissue products prepared according to the present invention may, in certain embodiments, have a sheet bulk of about 15.0 cc/g or greater, such as from about 15.0 to about 20 cc/g.

As used herein, the term “Slope” refers to the slope of the line resulting from plotting tensile versus stretch and is an output of the MTS TestWorks™ in the course of determining the tensile strength as described in the Test Methods section herein. Slope typically has units of kilograms (kg) and is measured as the gradient of the least-squares line fitted to the load-corrected strain points falling between a specimen-generated force of 70 to 157 grams (0.687 to 1.540 N).

As used herein, the term “Geometric Mean Slope” (GM Slope) generally refers to the square root of the product of machine direction slope and cross-machine direction slope. While the GM Slope may vary amongst tissue products prepared according to the present invention, in certain embodiments, tissue products may have a GM Slope less than about 15.00 kg, such as from about 10.00 to about 15.00 kg.

As used herein, the term “Geometric Mean Tensile” (GMT) refers to the square root of the product of the machine direction tensile strength and the cross-machine

direction tensile strength of the web. The GMT of tissue products prepared according to the present invention may vary, however, in certain instances the GMT may be about 2,500 g/3" or greater, such as about 3,000 g/3" or greater, such as about 3,200 g/3" or greater, such as from about 2,500 to about 3,500 g/3", such as from about 3,000 to about 3,400 g/3".

As used herein, the term "TEA Index" refers to the geometric mean tensile energy absorption (having units of g·cm/cm<sup>2</sup>) at a given geometric mean tensile strength (having units of grams per three inches) as defined by the equation:

$$\text{TEA Index} = \frac{\text{GM TEA (g} \cdot \text{cm/cm}^2\text{)}}{\text{GMT(g/3")}} \times 1,000$$

While the TEA Index may vary, in certain instances tissue products prepared according to the present invention have a TEA Index of about 10.0 or greater, such as from about 10.0 to about 12.0.

#### DETAILED DESCRIPTION

The present inventors have successfully balanced the manufacture of a molded, three-dimensional tissue sheet to create a multi-ply tissue product that is visually pleasing and has improved physical attributes. For example, the inventive multi-ply tissue products have improved cross-machine

about 14.0 percent or greater, such as from about 13.0 to about 15.0 percent. Surprisingly, the foregoing levels of CD stretch may be achieved even without creping the product and at relatively high degrees of CD tensile strength of about 2,500 g/3" or greater, such as about 2,750 g/3" or greater, such as about 3,000 g/3" or greater, such as from about 2,500 to about 3,750, such as from about 2,750 to about 3,500 g/3", such as from about 3,000 to about 3,300 g/3".

In other embodiments the tissue products of the present invention have good durability in the cross-machine direction, such as a CD TEA of about 25.0 g·cm/cm<sup>2</sup> or greater, such as about 28.0 g·cm/cm<sup>2</sup> or greater, such as about 30.0 g·cm/cm<sup>2</sup> or greater, such as from about 25.0 to about 34.0 g·cm/cm<sup>2</sup>. The foregoing CD TEA values may be achieved at CD tensile strengths from about 2,500 g/3" to about 3,750 g/3" and more preferably from about 3,000 to about 3,500 g/3". In this manner, the inventive tissue products may have a CD TEA Index of about 10.0 or greater, such as about 10.5 or greater, such as about 11.0 or greater, such as from about 10.0 to about 12.0.

A comparison of the CD properties of several inventive and commercially available tissue products may be found in Table 1, below. Compared to commercially available tissue products, the inventive tissue products have a high degree of CD stretch, low CD slope and a relatively high degree of CD tensile strength. These differences are further illustrated in FIGS. 1-3.

TABLE 1

| Description                 | Plies | TAD | Creped | GMT (g/3") | CD TEA (g · cm/cm <sup>2</sup> ) | CD Stretch (%) | CD Slope (kg) | CD Tensile (g/3") |
|-----------------------------|-------|-----|--------|------------|----------------------------------|----------------|---------------|-------------------|
| Viva Multisurface Cloth     | 2     | Y   | N      | 2922       | 22.15                            | 12.4           | 8.98          | 2662              |
| Plenty                      | 2     | N   | Y      | 3412       | 24.34                            | 9.4            | 18.27         | 3367              |
| Boulder Ultra Wave          | 2     | Y   | Y      | 3355       | 21.81                            | 8.2            | 20.59         | 3276              |
| Kirkland Signature          | 2     | Y   | Y      | 2794       | 21.35                            | 8.3            | 29.07         | 2719              |
| Brawny                      | 2     | Y   | Y      | 3410       | 26.08                            | 9.2            | 25.36         | 3458              |
| Bounty Essentials           | 2     | Y   | Y      | 2682       | 16.96                            | 9.1            | 11.70         | 2241              |
| Sparkle                     | 2     | N   | Y      | 2879       | 13.28                            | 5.7            | 33.63         | 2132              |
| Great Value Ultra Strong    | 2     | Y   | Y      | 4067       | 23.91                            | 6.3            | 40.13         | 3831              |
| Great Value Everyday Strong | 2     | Y   | Y      | 2279       | 7.97                             | 4.4            | 28.96         | 1539              |
| Presto                      | 2     | Y   | Y      | 3264       | 21.20                            | 8.6            | 20.67         | 3216              |
| Inventive                   | 2     | Y   | N      | 3358       | 28.45                            | 14.0           | 9.85          | 3179              |
| Inventive                   | 2     | Y   | N      | 3472       | 32.10                            | 14.0           | 10.70         | 3298              |
| Inventive                   | 2     | Y   | N      | 3289       | 28.05                            | 14.0           | 8.63          | 3103              |
| Inventive                   | 2     | Y   | N      | 3191       | 26.03                            | 13.9           | 9.37          | 2932              |
| Inventive                   | 2     | Y   | N      | 3248       | 28.38                            | 14.4           | 9.53          | 3093              |

direction (CD) properties such as improved CD tensile energy absorption (CD TEA), CD stretch and CD modulus.

In certain instances, the improvement in physical attributes is accompanied by an aesthetically pleasing pattern, such as a multi-ply tissue product having first and second patterns, where the first pattern is embossed, and the second pattern is unembossed. The first embossed pattern may cover a relatively minor percentage of the total surface area of the tissue product, such as less than about 15 percent and more preferably less than about 10 percent. Additionally, the embossed pattern may comprise discrete, non-linear line elements which consumers find visually appealing, particularly when the line elements are arranged in geometric patterns that give the product a cloth-like appearance.

Accordingly, in certain embodiments, the invention provides a multi-ply tissue product, particularly an embossed multi-ply product, having a CD stretch of about 13.0 percent or greater, such as about 13.5 percent or greater, such as

Accordingly, in certain embodiments, the inventive tissue products are both durable and flexible, particularly in the cross-machine direction. For example, multi-ply tissue products prepared according to the present invention have geometric mean tensile strength (GMT) of from about 2,500 to about 3,500 g/3", such as from about 3,000 to about 3,400 g/3" and a CD Slope of about 15.0 kg or less, such as about 12.0 kg or less, such as about 10.0 kg or less, such as from about 8.0 to about 12.0 kg. The relatively low degree of stiffness does not come at the expense of cross-machine direction durability. For example, the tissue products generally have CD tensile strengths from about 2,500 g/3" to about 3,750 g/3" and more preferably from about 3,000 to about 3,500 g/3" and a CD Stretch of about 13.0 percent or greater, such as about 13.5 percent or greater, such as about 14.0 percent or greater, such as from about 13.0 to about 15.0 percent.

Surprisingly, the improved cross-machine direction properties may be achieved without creping the tissue web.

Rather than crepe the web during manufacture, the instant tissue products may be produced by transferring a partially dewatered web to a transfer fabric having a high degree of topography to strain the nascent sheet in the cross-machine direction. In this manner, tissue products of the present invention may be manufactured by a process that employs a transfer fabric, particularly a transfer fabric that transfers the nascent tissue web from a forming fabric to a through-air drying fabric. Such fabrics may be employed in through-air drying (TAD) manufacturing processes. In particularly preferred embodiments tissue products are manufactured using a high topography transfer fabric and through-air drying fabric in an uncreped through-air dried (UCTAD) process.

With reference now to FIG. 4, a method for making through-air dried paper sheets is illustrated. Shown is a twin wire former having a papermaking headbox 34, such as a layered headbox, which injects or deposits a stream 36 of an aqueous suspension of papermaking fibers onto the forming fabric 38 positioned on a forming roll 39. The forming fabric serves to support and carry the newly-formed wet web downstream in the process as the web is partially dewatered to a consistency of about 10 dry weight percent. Additional dewatering of the wet web can be carried out, such as by vacuum suction, while the wet web is supported by the forming fabric.

The wet web is then transferred from the forming fabric to a transfer fabric 40. In one embodiment, the transfer fabric can be traveling at a slower speed than the forming fabric in order to impart increased stretch into the web. This is commonly referred to as a "rush" transfer. The relative speed difference between the two fabrics can be from 0 to 60 percent, more specifically from about 15 to 45 percent. Transfer is preferably carried out with the assistance of a vacuum shoe 42 such that the forming fabric and the transfer fabric simultaneously converge and diverge at the leading edge of the vacuum slot.

The transfer fabric preferably is a woven fabric having a relatively high degree of surface topography. The surface topography may be imparted by weaving the fabric such that the web contacting surface of the fabric has a plurality of continuous, substantially parallel, ridges separated from one another by valleys. The ridges may be oriented substantially in the machine-direction and may be straight or have a wave-like shape. In those instances where the ridges have a wave-like shape, they may be skewed slightly, such as from about 1 to about 2 degrees, relative to the machine direction. Further, the wave-like ridges may have a wavelength from about 4 to about 8 mm, such as from about 5 to about 6 mm. The upper surfaces of the ridges is preferably substantially smooth, while the valleys are smooth with small, uniform pores to facilitate draining of water from the nascent web and through the fabric.

A profilometry scan of one embodiment of a topographic transfer fabric useful in the present invention is shown in FIG. 5. The profilometry scan was obtained by scanning the fabric contacting surface of a fabric sample using an FRT MicroSpy® Profile profilometer (FRT of America, LLC, San Jose, CA) and then analyzing the image using Nanovea® Ultra software version 7.4 (Nanovea Inc., Irvine, CA). FIG. 5 illustrates the wave-like, substantially machine direction oriented, ridges 100 and valleys 102 disposed therebetween. The illustrated fabric was woven from warp and weft yarns having a similar diameter of about 0.30 mm. The yarns were woven to yield a fabric having valley depths, the vertical distance between the upper surface plane of the ridges and the bottom most surface plane of the web contacting surface of the fabric, of about 0.50 mm. Further, the yarns were

woven to produce a plurality of substantially parallel, wave-like ridges spaced apart from one another a distance of about 2.0 mm.

Generally, transfer fabrics useful in the present invention have relatively deep valleys, such as valleys having valley depths greater than about 0.50 mm, such as from about 0.50 to about 0.70 mm.

Valley depth may be measured by profilometry and is generally taken from a simulated base sheet generated by a 10 morphological closing filter. The valley depth is measured as the difference between C2 (95 percentile height) and C1 (5 percentile height) values, having units of millimeters (mm). In certain instances, valley depth may be referred to as S90. To determine valley depth a profilometry scan of a fabric is 15 generated and a histogram of the measured heights of the simulated base sheet is generated, and an S90 value (95 percentile height (C2) minus the 5 percentile height (C1), expressed in units of mm) is calculated.

The valley width of a given transfer fabric may vary 20 depending on the weave pattern, however, in certain instances the valley width may be greater than about 1.5 mm and still more preferably greater than about 2.0 mm, such as from about 1.5 to about 3.5 mm. The valley width may also be measured by profilometry. Scans obtained as described 25 above may be used to calculate the Psm value, having units of millimeters (mm).

Preferably the transfer fabrics of the present invention provide the nascent web with a relatively high degree of CD strain. Profilometry may again be used to determine the 30 degree of CD strain imparted by the transfer fabric to the nascent web. Profilometry scans obtained as described above may be used to calculate the PLo value, which is indicative of CD strain, and is preferably at least about 15 percent, more preferably at least about 16 percent and still 35 more preferably at least about 17 percent, such as from about 15 to about 19 percent.

With reference again to FIG. 4, the nascent web is transferred from the transfer fabric 40 to the through-air drying fabric 44 with the aid of a vacuum transfer roll 46 or 40 a vacuum transfer shoe, optionally again using a fixed gap transfer as previously described. The through-air drying fabric can be traveling at about the same speed or a different speed relative to the transfer fabric. If desired, the through-air drying fabric can be run at a slower speed to further 45 enhance stretch. Transfer can be carried out with vacuum assistance to ensure deformation of the sheet to conform to the through-air drying fabric, thus yielding desired bulk and imparting the web with a three-dimensional topographical pattern. Suitable through-air drying fabrics are described, for 50 example, in U.S. Pat. Nos. 6,998,024, 7,611,607 and 10,161, 084, the contents of which are incorporated herein by reference in a manner consistent with the present disclosure.

The level of vacuum used for the web transfers can be 55 from about 3 to about 15 inches of mercury (75 to about 380 millimeters of mercury), preferably about 5 inches (125 millimeters) of mercury. The vacuum shoe (negative pressure) can be supplemented or replaced by the use of positive pressure from the opposite side of the web to blow the web onto the next fabric in addition to or as a replacement for 60 sucking it onto the next fabric with vacuum. Also, a vacuum roll or rolls can be used to replace the vacuum shoe(s).

In certain preferred embodiments the through-air drying fabric is a woven fabric comprising a plurality of MD oriented protuberances, which may be continuous or discrete. In a particularly preferred embodiment the MD oriented protuberances are continuous and have a width of 65 from about 0.2 to about 2.5 mm, such as from about 0.5 to

about 2.0 mm and the frequency of occurrence of the MD oriented protuberances in the cross-machine direction of the fabric is from about 0.5 to about 8 per centimeter, such as from about 3.2 to about 7.9 per centimeter, such as from about 4.2 to about 5.3 per centimeter.

The MD oriented protuberances may be substantially aligned with the MD axis of the fabric or they may have a non-zero element angle. For example, the warp filaments may be woven to form protuberances extending in a continuous manner across the fabric and slightly skewed relative to the MD axis of the fabric. In this manner the MD oriented protuberances may have a non-zero element angle, such as an element angle from about 0.5 to 20 degrees, such as from about 2 to about 15 degrees, and more preferably from about 2 to about 10 degrees. In a particularly preferred embodiment, the web contacting surface of the fabric comprises a plurality of spaced apart, parallel, MD oriented protuberances having an element angle from about 2 to about 10 degrees.

In certain embodiments the MD oriented protuberances may be arranged in a continuous pattern, extending from a first lateral edge of the fabric to a second lateral edge, in which adjacent protuberances are generally parallel to one another and equally spaced apart. Between adjacent protuberances are valleys having sidewalls formed by the protuberances. In this manner, the valleys, like the protuberances, may be oriented at an angle relative to the MD axis of the fabric.

Papermaking fabrics having woven MD oriented protuberances suitable for use in the present invention may be prepared as described in U.S. Pat. Nos. 6,998,024 and 7,611,607, the contents of which are incorporated herein in a manner consistent with the present disclosure. In a particularly preferred embodiment, the MD oriented protuberances may be substantially continuous and woven from two or more warp filaments grouped together and supported by multiple shute strands of two or more diameters as disclosed in U.S. Pat. No. 7,611,607. MD protuberances woven in this manner can be oriented at an angle of from 0 to about 15 degrees relative to the true machine direction of the fabric.

The MD oriented protuberances can be configured substantially the same in terms of any one or more characteristics of height, width, length or element angle. For example, in certain embodiments, substantially all the MD oriented protuberances have substantially similar characteristics of height, width and element angle. In other embodiments however, the MD oriented protuberances may be configured such that one or more characteristics of height, width, or length of the protuberances vary from one MD oriented protuberance to another MD oriented protuberance.

In certain embodiments, in addition to MD oriented protuberances, the through-air drying fabric may comprise a plurality of second protuberances, which are generally oriented in the cross-machine direction and are preferably discrete. In particularly preferred embodiments the CD oriented protuberances are formed by topically applying a polymeric material to the woven support structure. Suitable methods of topical application include printing and extruding polymeric material onto the surface of the woven support structure. Particularly suitable polymeric materials include materials that can be strongly adhered to the woven support structure and are resistant to thermal degradation at typical tissue machine dryer operating conditions and are reasonably flexible, such as silicones, polyesters, polyurethanes, epoxies, polyphenylsulfides and polyetherketones.

In other embodiments the CD oriented protuberances may be formed by extruding a polymeric strand onto a woven

support structure, such as that described in U.S. Pat. No. 6,398,910, the contents of which are incorporated herein in a manner consistent with the present disclosure. In such embodiments the polymeric strand is applied so as to form a raised CD oriented protuberance above the upper most plane of the woven support structure. Alternative methods of forming the CD oriented protuberances include applying cast or cured films, weaving, embroidering or stitching polymeric fibers into the surface.

10 The CD oriented protuberances may be arranged on the web contacting surface of the fabric in a pattern. For example, the CD oriented protuberances may be discrete and occur in a regular, repeating pattern comprising pairs of protuberance, such as a first pair of protuberances and a second pair of protuberances, spaced apart from one another in the cross-machine direction (D1) at least about 5.0 mm and more preferably at least about 10.0 mm. Within a given pair of protuberances, the protuberances may be spaced apart a distance (D2) from about 2.0 to about 6.0 mm, such as from about 2.0 to about 5.0 mm.

15 In other embodiments the CD oriented protuberances may be arranged in a pattern such that each CD oriented protuberance contacts, and more preferably traverses, at least one MD oriented protuberance and in certain instances two or more adjacent MD oriented protuberances. In those embodiments where a CD protuberance contacts adjacent MD oriented protuberances, the CD protuberance may extend across the entire width of a valley and form a valley end wall.

20 While supported by the through-air drying fabric, the web is dried to a consistency of about 94 percent or greater by the through-air dryer 48 and thereafter transferred to a carrier fabric 50. The dried basesheet 52 is transported to the reel 54 using carrier fabric 50 and an optional carrier fabric 56. An optional pressurized turning roll 58 can be used to facilitate transfer of the web from carrier fabric 50 to fabric 56.

25 In one embodiment, the reel 54 can run at a speed slower than the fabric 56 in a rush transfer process for building bulk into the paper web 52. For instance, the relative speed difference between the reel and the fabric can be from about 5 to about 25 percent and, particularly from about 12 to about 14 percent. Rush transfer at the reel can occur either alone or in conjunction with a rush transfer process upstream, such as between the forming fabric and the transfer fabric.

30 In certain embodiments basesheets useful in forming tissue products of the present invention may comprise a single homogenous or blended layer or be multi-layered. In those instances where the basesheet is multi-layered it may comprise, two, three, or more layers. For example, the basesheet may comprise three layers such as first and second outer layers and a middle layer disposed there between. The layers may comprise the same or different fiber types. For example, the first and second outer layers may comprise short, low coarseness wood pulp fibers, such as hardwood kraft pulp fibers, and the middle layer may comprise long, low coarseness wood pulp fibers, such as northern softwood kraft pulp fibers.

35 In those instances where the web comprises multiple layers, the relative weight percentage of each layer may vary. For example, the web may comprise first and second outer layers and a middle layer where the first outer layer comprises from about 25 to about 35 weight percent of the layered web, the middle layer comprises from about 30 to about 50 weight percent of the layered web and the second outer layer comprises from about 25 to about 35 weight percent of the layered web. Multi-layered basesheets useful

## 11

in the present invention may be formed using any number of different processes known in the art, such as the process disclosed in U.S. Pat. No. 5,129,988, the contents of which are incorporated herein in a manner consistent with the present disclosure.

In certain instances, a layer or other portion of the web, including the entire web, can be provided with wet or dry strength agents. As used herein, "wet strength agents" are materials used to immobilize the bonds between fibers in the wet state. Any material that when added to a paper web or sheet at an effective level results in providing the sheet with a wet geometric tensile strength:dry geometric tensile strength ratio in excess of 0.1 will, for purposes of this invention, be termed a wet strength agent. Typically, these materials are termed either as permanent wet strength agents or as "temporary" wet strength agents. For the purposes of differentiating permanent from temporary wet strength, permanent will be defined as those resins which, when incorporated into paper or tissue products, will provide a product that retains more than 50 percent of its original wet tensile strength after exposure to water for a period of at least five minutes. Temporary wet strength agents are those which show less than 50 percent of their original wet strength after being saturated with water for five minutes. Both classes of material find application in the present invention. The amount of wet strength agent or dry strength added to the pulp fibers can be at least about 0.1 dry weight percent, more specifically about 0.2 dry weight percent or greater, and still more specifically from about 0.1 to about 3 dry weight percent, based on the dry weight of the fibers.

Particularly preferred wet strength agents include resin binder materials selected from the group consisting of polyamide-epichlorohydrin resins, polyacrylamide resins, and mixtures thereof. Of particular utility are the various polyamide-epichlorohydrin resins. These materials are low molecular weight polymers provided with reactive functional groups such as amino, epoxy, and azetidinium groups. Particularly useful polyamide-epichlorohydrin resins include those marketed under the tradename KYMENE (Solenis, Wilmington, DE).

Useful dry strength additives include carboxymethyl cellulose resins, starch based resins, and mixtures thereof. Examples of preferred dry strength additives include carboxymethyl cellulose, and cationic polymers from the ACCO chemical family (American Cyanamid Company of Wayne, NJ) such as ACCO 711 and ACCO 514.

Suitable temporary wet strength resins include, but are not limited to, those resins that have been developed by American Cyanamid and are marketed under the name PAREZ™ 631 NC wet strength resin (now available from Cytec Industries, located in West Paterson, NJ). This and similar resins are described in U.S. Pat. Nos. 3,556,932 and 3,556,933. Other temporary wet strength agents that should find application in this invention include modified starches such as those available from National Starch and marketed as CO BOND™ 1000 modified starch.

Although wet and dry strength agents as described above find particular advantage for use in connection with this invention, other types of bonding agents can also be used to provide the necessary wet resiliency. They can be applied at the wet end of the basesheet manufacturing process or applied by spraying or printing after the basesheet is formed or after it is dried.

The processes of the present invention may be useful in producing numerous and different tissue products particularly paper towels, napkins, industrial wipers, and the like. The instant multi-ply tissue product may be constructed

## 12

from two or more plies that are manufactured using the same or different tissue making techniques. In a particularly preferred embodiment the multi-ply tissue product comprises two thorough-air dried tissue plies where each ply has a basis weight greater than about 20 gsm, such as from about 20 to about 50 gsm, such as from about 22 to about 30 gsm, where the plies have been attached to one another by a glue laminating embossing process which provides the tissue product with an embossing pattern on at least one of its outer surfaces.

In one embodiment of the present invention, the tissue product has a plurality of embossments. In one embodiment the embossment pattern is applied only to the first ply, and therefore, each of the two plies serve different objectives and are visually distinguishable. For instance, the embossment pattern on the first ply provides, among other things, improved aesthetics regarding thickness and quilted appearance, while the second ply, being unembossed, is devised to enhance functional qualities such as absorbency, thickness and strength. In another embodiment the fibrous structure product is a two-ply product wherein both plies comprise a plurality of embossments. Suitable means of embossing include, for example, those disclosed in U.S. Pat. Nos. 5,096,527, 5,667,619, 6,032,712 and 6,755,928.

In certain embodiments the embossed area may be about 15 percent or less, such as 12 percent or less, such as 10 percent or less, such as from about 4 to about 10 percent or from about 5 to about 8 percent. In addition to the plurality of embossments the tissue product has a first surface comprising a plurality of substantially machine direction (MD) oriented ridges that are spaced apart from one another and define valleys there between. The substantially machine direction oriented ridges may be spaced apart from one another such that the background pattern comprises one or more ridges every 10 cm, such as from 10 to about 60 ridges every 10 cm, such as from about 30 to about 50 ridges every 10 cm, as measured along the cross-machine direction axis.

In a particularly preferred embodiment, the embossments may be in the form of discrete, non-linear elements that form recognizable shapes, such as a V-shape. The non-linear elements may be arranged into motifs that may be further arranged to form a pattern, such as the illustrated chevron pattern. While in certain embodiments the embossments may form recognizable shapes, such as letters or geometric shapes, such as a triangle, diamond, trapezoid, parallelogram, rhombus, star, pentagon, hexagon, octagon, or the like, the invention is not so limited. In other embodiments the embossments may comprise non-linear elements which are arranged, but do not form a recognizable geometric shape.

## Test Methods

## Profilometry

Fabric properties are generally measured using a non-contact profilometer as described herein. To prevent any debris from affecting the measurements, all images are subjected to thresholding to remove the top and bottom 0.5 mm of the scan. To fill any holes resulting from the thresholding step and provide a continuous surface on which to perform measurements, non-measured points are filled. The image is also flattened by applying arightness filter. Finally, a base sheet simulation is obtained using morphological filtering.

Profilometry scans of the fabric contacting surface of a sample were created using an FRT MicroSpy® Profile

profilometer (FRT of America, LLC, San Jose, CA) and then analyzing the image using Nanovea® Ultra software version 7.4 (Nanovea Inc., Irvine, CA). Samples were cut into squares measuring 145×145 mm. The samples were then secured to the x-y stage of the profilometer using an aluminum plate having a machined center hole measuring 2×2 inches, with the fabric contacting surface of the sample facing upwards, being sure that the samples were laid flat on the stage and not distorted within the profilometer field of view.

Once the sample was secured to the stage the profilometer was used to generate a three-dimensional height map of the sample surface. A 1602×1602 array of height values were obtained with a 30  $\mu\text{m}$  spacing resulting in a 48 mm MD×48 mm CD field of view having a vertical resolution 100 nm and a lateral resolution 6  $\mu\text{m}$ . The resulting height map was exported to .sdf (surface data file) format.

Individual sample .sdf files were analyzed using Nanovea® Ultra version 7.4 by performing the following functions:

- (1) Using the “Thresholding” function of the Nanovea® Ultra software the raw image (also referred to as the field) is subjected to thresholding by setting the material ratio values at 0.5 to 99.5 percent such that thresholding truncates the measured heights to between the 0.5 percentile height and the 99.5 percentile height;
- (2) Using the “Fill in Non-Measured Points” function of the Nanovea® Ultra software the non-measured points are filled by a smooth shape calculated from neighboring points;
- (3) Using Robust Gaussian filter roughness filter with a cut off wavelength of 24.0 mm and selecting “manage end effects”;
- (4) Using the “Morphological Filtering” selecting “closing filter and a structuring element of a sphere with a 1.7 mm diameter”;
- (5) Using the “Abbott-Firestone Curve” study function of the Nanovea® Ultra software an Abbott-Firestone Curve is generated from which “interactive mode” is selected and a histogram of the measured heights is generated, from the histogram an S90 value (95 percentile height (C2) minus the 5 percentile height (C1), expressed in units of mm) is calculated.
- (6) Using “convert surface into series of profiles” and data from “parameters table”.

Based upon the foregoing, three values, indicative of the fabric topography are reported—valley depth, valley width and strain. Valley width is the Psm value having units of millimeters (mm). Valley depth is the difference between C2 and C1 values and has units of millimeters (mm). In certain instances, pocket depth may be referred to as 590. Strain is the PLo value having units of percent (%).

#### Basis Weight

Prior to testing, all samples are conditioned under TAPPI conditions (23±1° C. and 50±2 percent relative humidity) for a minimum of 4 hours. Basis weight of sample is measured by selecting twelve (12) products (also referred to as sheets) of the sample and making two (2) stacks of six (6) sheets. In the event the sample consists of perforated sheets of bath or towel tissue, the perforations must be aligned on the same side when stacking the usable units. A precision cutter is used to cut each stack into exactly 10.16×10.16 cm (4.0×4.0 inch) squares. The two stacks of cut squares are combined to make a basis weight pad of twelve (12) squares thick. The basis weight pad is then weighed on a top loading

balance with a minimum resolution of 0.01 grams. The top loading balance must be protected from air drafts and other disturbances using a draft shield. Weights are recorded when the readings on the top loading balance become constant. The mass of the sample (grams) per unit area (square meters) is calculated and reported as the basis weight, having units of grams per square meter (gsm).

#### Caliper

Caliper is measured in accordance with TAPPI Test Method T 580 pm-12 “Thickness (caliper) of towel, tissue, napkin and facial products.” The micrometer used for carrying out caliper measurements is an Emveco 200-A Tissue Caliper Tester (Emveco, Inc., Newberg, OR). The micrometer has a load of 2 kilo-Pascals, a pressure foot area of 2,500 square millimeters, a pressure foot diameter of 56.42 millimeters, a dwell time of 3 seconds and a lowering rate of 0.8 millimeters per second.

#### Tensile

Tensile testing is conducted on a tensile testing machine maintaining a constant rate of elongation and the width of each specimen tested is 3 inches. Testing is conducted under TAPPI conditions. More specifically, samples for dry tensile strength testing were prepared by conditioning under TAPPI conditions for at least 4 hours and then cutting a 3±0.05 inch (76.2±1.3 mm) wide strip in either the machine direction (MD) or cross-machine direction (CD) orientation using a JDC Precision Sample Cutter (Thwing-Albert Instrument Company, Philadelphia, PA, Model No. JDC 3-10, Serial No. 37333) or equivalent. The instrument used for measuring tensile strengths was an MTS Systems Sintech 11S, Serial No. 6233. The data acquisition software was MTS TestWorks® for Windows Ver. 3.10 (MTS Systems Corp., Research Triangle Park, NC). The load cell was selected from either a 50 Newton or 100 Newton maximum, depending on the strength of the sample being tested, such that the majority of peak load values fall between 10 to 90 percent of the load cell’s full-scale value. The gauge length between jaws was 4±0.04 inches (101.6±1 mm) for facial tissue and towels and 2±0.02 inches (50.8±0.5 mm) for bath tissue. The crosshead speed was 10±0.4 inches/min (254±1 mm/min), and the break sensitivity was set at 65 percent. The sample was placed in the jaws of the instrument, centered both vertically and horizontally. The test was then started and ended when the specimen broke. The peak load was recorded as either the “MD tensile strength” or the “CD tensile strength” of the specimen depending on direction of the sample being tested. Ten representative specimens were tested for each product or sheet and the arithmetic average of all individual specimen tests was recorded as the appropriate MD or CD tensile strength having units of grams per three inches (g/3"). Tensile energy absorbed (TEA) and slope are also calculated by the tensile tester. TEA is reported in units of g·cm/cm<sup>2</sup> and slope is recorded in units of kilograms (kg). Both TEA and Slope are directionally dependent and thus MD and CD directions are measured independently. All products were tested in their product forms without separating into individual plies.

#### Examples

Basesheets were made using a through-air dried paper-making process commonly referred to as “uncreped through-air dried” (“UCTAD”) and generally described in U.S. Pat.

No. 5,607,551, the contents of which are incorporated herein in a manner consistent with the present disclosure. The basesheets were then converted by calendering, slitting and winding to yield single ply tissue products.

In all cases basesheets were produced from a furnish comprising northern softwood kraft (NSWK) and eucalyptus hardwood kraft (EHWK) using a layered headbox fed by three stock pumps such that the webs having three layers (two outer layers and a middle layer) were formed. Composition of the basesheet is described in Table 2, below. The two outer layers comprised EHWK (each layer comprising 20 wt % of the tissue web) and the middle layer comprised NSWK (middle layer comprised 60 wt % of the tissue web). Strength was controlled via the addition of carboxymethyl-cellulose (CMC) and permanent wet strength resin, and/or by refining the furnish.

TABLE 2

| Fabric Layer Furnish (wt %) | Middle Layer Furnish (wt %) | Air Layer Furnish (wt %) | Permanent Wet Strength (kg/MT) | Dry Strength (kg/MT) |
|-----------------------------|-----------------------------|--------------------------|--------------------------------|----------------------|
| 20                          | 60                          | 20                       | 6                              | 2                    |

Each furnish was diluted to approximately 0.2 percent consistency and delivered to a layered headbox and deposited on a Voith Fabrics TissueForm V forming fabric (commercially available from Voith Fabrics, Appleton, WI). The wet web was vacuum dewatered to approximately 25 percent consistency and then transferred to a transfer fabric. Inventive samples were transferred to the fabric depicted in FIG. 5 and described further in Table 3, below. The transfer fabric used to produce the control samples is also described in Table 3, below. Both transfer fabrics are commercially available from Voith Fabrics, Appleton, WI.

TABLE 3

|           | S90 (mm) | Psm (mm) | PLo (%) | Air Permeability (CFM) | Fabric Caliper (mm) | MD Oriented Ridges per 48 mm |
|-----------|----------|----------|---------|------------------------|---------------------|------------------------------|
| Inventive | 0.56     | 2.03     | 18.0    | 360                    | 1.46                | 24                           |
| Control   | 0.66     | 2.66     | 15.8    | 479                    | 1.71                | 18                           |

The web was transferred from the transfer fabric to a through-air drying fabric substantially as described in co-pending U.S. patent application Ser. No. 16/205,355, the contents of which are incorporated herein in a manner consistent with the present disclosure. The through-air drying fabric consisted of a woven base fabric (t1205-2 woven fabric, commercially available from Voith Fabrics, Appleton, WI and previously described in U.S. Pat. No. 8,500,955). The woven base fabric had a plurality of spaced apart substantially continuous machine direction (MD) oriented protuberances that defined plurality of valleys there between. The fabric further comprised a plurality of discrete, non-woven, cross-machine direction (CD) oriented protuberances. The discrete, non-woven, cross-machine direction (CD) oriented protuberances comprised a silicone printed onto the base fabric and covered approximately 7.5 percent of the web contacting surface of the fabric.

The nascent web was rush transferred to the through-air drying fabric at a rush transfer rate of about 28 percent. The web was through-air dried while supported by the through-air drying fabric to yield a dried basesheet. The dried basesheet was converted into a spirally wound two-ply towel

product by first calendering the basesheet. Basesheet was calendered using a single calender unit comprising a patterned steel roll and a 40 P&J polyurethane roll. The calenders were configured substantially as described in U.S. Pat. No. 10,040,265, the contents of which are incorporated herein in a manner consistent with the present invention. Loading of the calender ranged from about 40 pounds per linear inch (pli) to about 250 pli. The calendered base sheet was further converted by embossing and laminating two plies together. The two-ply tissue product was then converted into a rolled towel product and subjected to physical testing, the results of which are shown in Tables 4 and 5, below.

TABLE 4

| Sample      | Description         | Basis Weight (gsm) | Caliper (μm) | Sheet Bulk (cc/g) | GMT (g/3") | GM Stretch (%) |
|-------------|---------------------|--------------------|--------------|-------------------|------------|----------------|
| Control     | Viva MSC VR CAS 58  | 51.6               | 960          | 18.6              | 3846       | 14.0           |
| Inventive 1 | Viva MSC VDR CAS 54 | 50.5               | 1010         | 20.0              | 3358       | 14.7           |
| Inventive 2 | Viva MSC VR CAS 58  | 51.2               | 1059         | 20.7              | 3472       | 14.6           |
| Inventive 3 | Viva MSC BR CAS 83  | 50.7               | 1048         | 20.7              | 3289       | 14.8           |
| Inventive 4 | Viva MSC DR CAS 110 | 49.6               | 880          | 17.8              | 3191       | 14.3           |
| Inventive 5 | Viva MSC HR CAS 165 | 50.4               | 880          | 17.4              | 3248       | 14.4           |

TABLE 5

| Sample      | CD Tensile (g/3") | CD TEA (g · cm/cm <sup>2</sup> ) | CD Stretch (%) | CD Slope (kg) | CD TEA Index |
|-------------|-------------------|----------------------------------|----------------|---------------|--------------|
| Control     | 3651              | 30.90                            | 12.1           | 14.10         | 8.46         |
| Inventive 1 | 3179              | 28.45                            | 14.0           | 9.85          | 8.95         |
| Inventive 2 | 3298              | 32.10                            | 14.0           | 10.70         | 9.73         |
| Inventive 3 | 3103              | 28.05                            | 14.0           | 8.63          | 9.04         |
| Inventive 4 | 2932              | 26.03                            | 13.9           | 9.37          | 8.88         |
| Inventive 5 | 3093              | 28.38                            | 14.4           | 9.53          | 9.18         |

What is claimed is:

1. A rolled tissue product comprising an embossed multi-ply tissue web spirally wound about a core, the multi-ply web comprising a plurality of embossments and having a cross-machine direction (CD) tensile of from 2,500 to 3,750 g/3" or greater, a CD TEA from about 25.0 to about 35.0 g·cm/cm<sup>2</sup> and a CD Slope from about 7.5 to about 15.0 kg.
2. The rolled tissue product of claim 1 wherein the multi-ply web has a geometric mean tensile strength (GMT) from about 2,500 to about 3,500 g/3".
3. The rolled tissue product of claim 1 wherein the multi-ply web has a geometric mean tensile (GMT) from about 3,000 to about 3,400 g/3".
4. The rolled tissue product of claim 1 wherein the multi-ply web has a basis weight from about 46.0 to about 52.0 grams per square meter (gsm).
5. The rolled tissue product of claim 4 wherein the multi-ply web has a sheet bulk greater than about 15 cubic centimeters per gram (cc/g).
6. The rolled tissue product of claim 1 wherein the multi-ply web has a CD Stretch from about 13.0 to about 15.0 percent.

7. The rolled tissue product of claim **1** wherein the multi-ply web has a sheet bulk from about 15.0 to about 20 cc/g.

8. The rolled tissue product of claim **1** wherein the multi-ply web has a geometric mean slope (GM Slope) from 5 about 10.00 to about 15.00 kg.

9. The rolled tissue product of claim **8** wherein the multi-ply web has a geometric mean tensile strength (GMT) from about 2,500 to about 3,500 g/3".

**10.** The rolled tissue product of claim **1** wherein the 10 multi-ply web has a TEA Index of about 10.0 or greater.

**11.** The rolled tissue product of claim **1** wherein the multi-ply web has a TEA Index from about 10.0 to about 12.0.

**12.** The rolled tissue product of claim **1** wherein the 15 multi-ply web is through-air dried.

**13.** The rolled tissue product of claim **1** wherein the multi-ply web is through-air dried and uncreped.

\* \* \* \* \*